

# UNITED STATES PATENT OFFICE.

FRANZ KOCH, OF GÖRLITZ, GERMANY, ASSIGNOR, BY MESNE ASSIGNMENTS, TO THE CHEMICAL FOUNDATION, INC., A CORPORATION OF DELAWARE.

## PROCESS FOR REMOVING FAT FROM RAW WOOL OR ANALOGOUS MATERIALS BY THE AID OF FAT SOLVENTS.

1,358,163.

Specification of Letters Patent.

Patented Nov. 9, 1920.

No Drawing.

Application filed February 3, 1914. Serial No. 816,391.

To all whom it may concern:

Be it known that I, Dr. FRANZ KOCH, engineer, a subject of the German Emperor, and a resident of Görlitz, in the Kingdom of Prussia, German Empire, have invented an Improvement in Processes for Removing Fat from Raw Wool or Analogous Materials by the Aid of Fat Solvents, of which the following description is a specification.

10 This invention relates to a novel process for eliminating or removing fat from raw wool or analogous materials. The invention will best be understood from the following description of one manner of carrying it into effect, the scope of the invention being more particularly pointed out in the appended claims.

15 The organic fat solvents heretofore used for the removal of fat from raw wool or analogous materials all had this disadvantage that, owing to the removal of fat from the individual fibers being carried too far, the treatment was liable to render the material brittle whereby its value was appreciably impaired.

20 In the case of raw wool, for example, from which after the removal of the yolk or wool fat the sweat excreta must also be eliminated or removed, the fibers in addition to the liability of becoming brittle also tend to turn yellow as a result of the penetration of the sweat lye or liquor into the cavities existing or thus produced in the individual fibers.

25 The present invention is based upon the knowledge that some chlorinated hydrocarbons of the fatty series and more particularly ethylene dichlorid and trichlorid, possess the wholly unexpected and useful property of dissolving to a very small extent only the fatty and waxlike substances which are present in the interior of the fibers either as a natural result of growth or from having subsequently penetrated 30 therein. For example, wool can be treated for a long time with hot ethylene trichlorid without impairing the pliability of the fibers by reason of the drying up of the fat. It will of course be understood that in order to obtain the best results, the temperature and the duration of the treatment must be regulated in accordance with the nature of the solvent and the nature of the fibrous material treated. The ready 35 solubility and miscibility of the fatty substances in question enable the fat to be

speedily removed or eliminated at low temperatures. Extremes of time and of temperature, therefore, play no part in the technical or practical execution of this improved 60 process.

65 The property above referred to as possessed by certain chlorinated hydrocarbons of the fatty series appears to be attributable to the fact that while these solvents dissolve the fat or oil that is upon the outer surface of the fibers, they, owing to their high specific gravity and molecular weight, do not penetrate into the microscopical interstices and the interior of the fibers.

70 The use of these substances substantially in accordance with any one of the usual fat removing and washing processes by the aid of chemical solvents in which the recovery of the means employed is aimed at, 75 furnishes a really effective method for freeing fibrous materials from fat. By means of the present invention, the yolk or wool oil can be removed from the surface of the raw wool fibers without previously lixiviating the sweat excreta and in such manner that the removal of such impurities as are soluble in water and others can be effected without the use of soap or soda. That is to say the present invention contemplates more particularly the use of ethylene dichlorid or trichlorid as solvents without the addition of soap, soda or other agents for emulsifying the solvent or rendering it soluble 80 in water, as has been commonly done here- 85 tofore. The use of the solvent in this manner renders its recovery after use a comparatively easy matter. Where the present invention is used there is no tendency whatever of the wool to turn yellow and the wool 90 retains to the fullest extent its natural fat or oil and its original pliability.

95 It will be apparent that the chlorinated bodies referred to can be used not only for all kinds of wool but also for all fibrous 100 and analogous materials such as cotton waste, hair, feathers, bristles and the like from the outer surface of which it is desired to remove waxy or fatty substances while allowing substances of the same kind that may be present in their interior to remain 105 there.

110 As one illustrative carrying out of the process the following may serve:

The wool can be spread out or distributed upon a sieve-like or other perforated surface in a suitable receptacle, and a circulating

flow of ethylene di- or trichlorid is then conducted through the wool, whereby the soluble constituents are dissolved. When all soluble constituents have been removed 5 the chlorinated hydrocarbon is drawn off. Preferably the wool is then rinsed with fresh di- or trichlorid of ethylene, and then by the introduction of steam or hot air the solvent adhering to the wool may be evaporated and, if desired, reclaimed.

From the foregoing it will be seen that the present process possesses many advantages over those heretofore used. By mixing these chlorinated bodies with other fat 15 solvents of lower specific gravity, the specific gravity and the cost per unit of volume may be reduced. The properties of such a mixture will represent approximately a mean of the properties of the different constituents according to the proportions in 20 which they are used.

Claims:

1. A process for removing fat or oil from raw wool or similar fibrous material, characterized by treating said fibrous material 25 with a chlorinated hydrocarbon of the fatty series as the solvent, in the absence of soap, soda or other agent for emulsifying the solvent or rendering it soluble in water.

2. A process for removing fat or oil from 30 raw wool or similar fibrous material, characterized by treating said fibrous material with ethylene dichlorid, in the absence of soap, soda or other agent for emulsifying the solvent or rendering it soluble in water. 35

In testimony whereof I have signed my name to this specification in the presence of two subscribing witnesses.

DR. ING. FRANZ KOCH.

Witnesses:

ALBERT PAUL,  
IDA PAUL GEB. KOCH.